

## UNITED STATES PATENT OFFICE

2,381,435

## GRAIN SHAPE CONTROL IN KILLED DEEP DRAWING MATERIALS

Robert S. Burns, Middletown, and Arthur S. McCabe, Seven Mile, Ohio, assignors to The American Rolling Mill Company, Middletown, Ohio, a corporation of Ohio

No Drawing. Application August 3, 1940,  
Serial No. 351,130

8 Claims. (Cl. 148—12)

In Patent No. 2,069,758, issued February 9, 1937, Hayes and Griffis have described the preparation of a deep drawing iron or steel which is non-aging, particularly in that it is free from the tendency to redevelop a definite yield point after the yield point has once been destroyed therein. The iron or steel is of a killed character, thoroughly deoxidized, and containing residual deoxidizer of the nature of aluminum or titanium. It is also free from blue brittleness. The non-aging feature of the material is attained through the characteristics mentioned above and a stabilizing heat treatment.

It will be understood that the provision of a deep drawing sheet in which the yield point, having once been destroyed by cold straining, will not return, so that the sheet may be stored indefinitely and still retain its deep drawing characteristics, has proved to be of tremendous importance in the art. The fundamental object of the present invention is to enhance the deep drawing characteristics of iron or mild steels of the Hayes and Griffis type, while retaining the other advantageous characteristics of their sheet.

Particular objects of our invention are the provision of a killed, non-aging, deep drawing iron or mild steel having not only unusual drawing properties, but freedom from surface difficulties, the provision of a material of the class referred to having the excellent drawing properties of material characterized by large grains, and the freedom from surface coarsening characteristic of materials having small grains.

These and other objects of our invention which will be set forth hereinafter or will be apparent to one skilled in the art upon reading these specifications, we accomplish by those treatments and in those products of which we shall now describe certain exemplary embodiments.

Stabilized, non-aging steels as currently manufactured have an analysis including components of the following order: carbon up to .08%, manganese .15 to .40% with copper and sulphur as low as possible, and containing after deoxidation, residual metallic aluminum in the range of .02 to .08%. It will be understood that these analyses are not limiting but are given as an example of successful commercial practice. For example, in the light of the teachings of the Hayes and Griffis patent, titanium or other materials may be employed in the place of the aluminum.

The killed steel is hot rolled to a gauge of the general order of .10 inch, depending upon the final gauge, and is then cold reduced about 50% and is box annealed, at temperatures ranging

from 1200 to 1400° F., whence it is slowly cooled and temper rolled. The box annealing and cooling constitute a thermal stabilizing treatment, and the resultant sheets are non-aging.

5 We have discovered that the deep drawing characteristics of killed, non-aging iron or mild steels may be improved by treatments which tend to produce a peculiar grain structure. Deep drawing materials should have a relatively low yield point, a relatively high elongation, a relatively low Rockwell hardness value and relatively high Olsen ductility test, these tests being standard tests of the A. S. T. M. These tests taken together are indicative of deep drawing equality but are not conclusive, nor is the composition, taken alone. Among other factors, the grain size of deep drawing metals has been found to be of great importance. A material characterized by a large grain size is in general capable of taking deep draws; but such materials are susceptible to an undesirable coarsening of the surface when drawn. These defects are not characteristic to the same extent of materials having a small grain size; but a fine grained material is 10 in general not as drawable.

15 We have stated that by certain treatment and manipulations in the process of making materials of the Hayes and Griffis type we can attain an unusual grain shape. This shape may be roughly described as spheroidal or pancake shape, the projection of the grains on planes longitudinal and transverse to the rolling direction showing the grain to be flattened. The flattened grains are so orientated that their dimensions 20 in the plane of the rolled sheet are greater than their dimension normal to the plane of the sheet. In other words the grain in our materials has assumed the shape of an oblate spheroid whose vertical axis (perpendicular to the sheet surface) is shorter than either of its horizontal axes. It 25 is to be understood, of course, that as in any aggregate of metallic grains the grain surfaces are not regularly formed and smoothly curved.

30 The type of grain structure to which we have referred is sharply distinguished on the one hand from a rounded grain structure or a structure in which the axes of the grains in all directions are substantially equal, which previously has been considered to be the ideal condition, but which material is of inferior drawing quality. It is to be distinguished on the other hand from that elongation of grains in the rolling direction only which results from cold rolling with insufficient annealing. This latter material is characterized 35 by having only the grain axes parallel to the

rolling direction elongated so that the grains are roughly cigar shaped. It is a material of very poor drawing quality. The appearance of the flattened or spheroidal grain characteristic of our products is associated with the treatment of the hot rolled material or thin bar ahead of the cold reduction and is attained as we shall now set forth.

The essential condition in securing our new type of grain is a pre-treatment, prior to the cold rolling in which the material has a controlled cooling in steps from a temperature range of 1525 to 1650° F. or higher. The temperature with respect to which the controlled cooling is practiced may be attained as the finishing temperature of hot rolling, or it may otherwise be attained as will be set forth hereinafter.

As an exemplary practice under our invention, a steel containing up to .08% carbon, substantially .15 to .40% manganese with low copper and sulphur is deoxidized (killed) with aluminum; and aluminum is added in such an amount as to result in a residual amount of aluminum in the steel of the order of .02 to .08%. Ingots of this composition are then hot rolled to some thickness in the neighborhood say of .10 inch, finishing the rolling operation in the range of 1525 to 1650° F. or higher. The material, if in strip sheet form, is cooled in air, or more rapidly, to a temperature substantially between 1100 to 1375° F. and then is coiled, whence it cools more slowly to room temperature. If the material is in sheet rather than in strip sheet form, substantially between 1100 to 1375° F. in the cooling cycle the cooling rate may be retarded in any way desired, as for example by stacking the sheets. Instead of coiling or stacking, the cooling of the material may be retarded to a similar extent by any other procedure.

The material is next cold reduced, the reduction being of the order of 50%, and may vary from 30 to 70% so that the material is of the desired gauge.

It is then box or close annealed at 1250 to 1400° F. for four or more hours and is cooled to room temperature at a relatively slow rate which for best results will be of the order of about 25° per hour, whence it is temper rolled to prevent stretcher straining.

It will be noted that of these factors, the composition of the metal and the deoxidation resulting in killing the steel and the leaving of residual deoxidizer therein, together with hot and cold reduction and the final annealing, are characteristic of the teachings of Hayes and Griffis; but the finishing of the hot rolling in the temperature range of 1525 to 1650° F. or higher, and the controlled cooling from that point preparatory to the cold rolling constitute additional features, which, when combined with the other steps, produce the peculiar grain condition to which we have referred.

The finishing of the material at a temperature of from 1525 to 1650° F. or higher, and the coiling of it at a temperature substantially between 1100 to 1375° F. has the effect of giving to the material a rapid cool simulating a quench from the higher temperature to substantially between 1100 to 1375° F. and a slow cool from that temperature to room temperature.

We have found that killed steels made as described, and having the flattened or spheroidal grain characteristic of our materials, are not only non-aging but have deep drawing qualities which are superior to those of freshly tempered rim-

ming steel. The action is peculiar to killed steel; and the same finishing temperature and cooling treatment applied to rimming steels will not produce it. The amount of distortion or flattening of the grains varies from a ratio of one for the vertical axis to one and one-half for both horizontal axes, to one for the vertical axis to four for both horizontal axes. Although there appears to be a variation in grain size within the steel, each grain has the characteristic flattened spheroidal shape. Moreover, though the grain size in the plane of the sheet is relatively coarse, the surface of the sheet after stretching or drawing is definitely superior in smoothness to materials otherwise produced, and is not by any means as rough as the grain size in the plane of the sheet would indicate from experience with steels manufactured and processed by conventional practice.

A material of the analysis above set forth and treated as described, showed a yield point of 22,500, a tensile strength of 43,700, an elongation of 45.0, a Rockwell hardness of 39 and an Olsen ductility value of .450 inch. In this material the ratio of the vertical axis to each of the horizontal axes of the grains was one to two, which is our preferred ratio.

The effects characteristic of our invention are not, so far as we have been able to ascertain, attainable by substantially different temperatures. For example, finishing the hot rolling at too low a temperature, namely a temperature somewhat below 1400° F., gives a grain structure elongated in the rolling direction only, which material has very poor drawing qualities. Material identical in formula to the first mentioned example when so treated gave a grain in which the ratio of the vertical axis to the horizontal axis transverse to the direction of rolling was one to one while the ratio of the vertical axis to the horizontal axis in the direction of rolling was one to four. While such material had a satisfactory yield point and a very low Rockwell value, it had a low percentage of elongation and poor drawing quality. Regardless of hot mill finishing temperature, a fast normalize (cooling rate approximately 300°/min.) of the thin bar ahead of the cold reduction and stabilizing heat treatment gave a material in which the ratio of the vertical axis to both horizontal axes was one to one. This material had a lower elongation, a higher yield point, and definitely poorer drawing qualities than our new material. It was a material finished at or slightly under 1400° F. from the hot rolling; but the same fast normalizing treatment applied to a material on which the hot rolling was finished at 1600° F. gave the same grain axis ratio, an even higher yield point, and an even lower elongation, and had very poor drawing qualities.

Having thus described our invention, what we claim as new and desire to secure by Letters Patent, is:

1. A process of producing a deep drawing iron or mild steel sheet or strip stock, which comprises hot rolling a killed iron or mild steel stock, finishing the hot rolling at a temperature in the range of substantially 1525 to 1650° F., rapidly cooling the stock in air from said temperature range to substantially between 1100 to 1375° F. and then more slowly cooling it to a cold rolling temperature, cold rolling the stock with a reduction of the order of 50%, and thereafter giving the stock a thermal stabilizing treatment, by heating said stock to a temperature below the

A<sub>3</sub> point and preferably in the neighborhood of the A<sub>1</sub> point and then cooling said stock sufficiently slowly to establish freedom from the unstable condition in the ferrite which gives rise to overstrain aging.

2. A killed iron or mild steel for deep drawing characterized by a grain structure in which the grain axis normal to the plane of the stock is less in dimension than both grain axes in the plane of the stock.

3. A deep drawing iron or mild steel strip or sheet stock containing carbon not to exceed substantially .08%, manganese substantially of the order of .15 to .40%, copper and sulphur being low, with metallic aluminum substantially of the order of .02 to .08%, balance substantially all iron, said stock being free from a tendency to re-develop a yield point when the yield point therein has been destroyed by cold straining, and further characterized by a grain shape in which the grain axis normal to the plane of the stock is less in dimension than both axes in the plane of the stock.

4. A deep drawing iron or mild steel strip or sheet stock containing carbon not to exceed substantially .08% manganese substantially of the order of .15 to .40%, copper and sulphur being low, with metallic aluminum substantially of the order of .02 to .08%, balance all iron, said stock being free from a tendency to re-develop a yield point when the yield point therein has been destroyed by cold straining, and further characterized by a grain shape in which the grain axis normal to the plane of the stock is less in dimension than both axes in the plane of the stock, said material having deep drawing characteristics with a drawability characteristic of coarse grained material and surface effects characteristic of a fine grained material.

5. Killed iron or mild steel strip or sheet stock for deep drawing characterized by high ductility and excellent surface when drawn and

further characterized by grain dimensions which, measured normal to the plane of the stock are characteristic of fine grain materials and measured in either direction in the plane of the stock are characteristic of coarse grained materials.

6. A process of producing a deep drawing iron or mild steel sheet or strip stock, which comprises thoroughly deoxidizing iron or mild steel with the employment of sufficient deoxidizing metal of the character of titanium and aluminum to leave residual deoxidizer in the metal, hot rolling the metal to thin bar, finishing the hot rolling of the thin bar at a temperature of substantially 1525 to 1650° F., cooling the hot rolled material at least as rapidly as in air to a temperature of the order of 1100 to 1375° F., retarding the cooling thereof by juxtaposing cooling portions of the metal to each other by coiling or stacking so as more slowly to cool the metal to cold rolling temperature, then cold rolling the metal to gauge with a reduction of the order of 50%, and thereafter annealing the material at a temperature in the range of 1250 to 1400° F., and slowly cooling it.

7. A process as set forth in claim 6 in which the metal as hot rolled contains a maximum carbon of the order of .08%, manganese of the order of .15 to .40% is low in copper and sulphur and contains residual deoxidizer of the order of .02% to .08%, balance being iron.

8. A killed iron or mild steel sheet or strip stock for deep drawing, characterized by grain structure in which a preponderance of the grains are of a flattened shape, such that a typical grain has its two axes in the plane of the stock of such a length that each is from one and one-half to four times as long as the axis of such grain normal to the plane of the stock.

ROBERT S. BURNS.  
ARTHUR S. McCABE.